

June 12, 1956

R. A. MILLER

2,750,332

METHOD AND APPARATUS FOR ELECTRO-DEPOSITION OF A LAYER  
OF UNIFORM THICKNESS ON A CONDUCTIVE SURFACE

Filed June 4, 1952



*Fig. 2*



*Fig. 3*



*Fig. 5*



INVENTOR.

BY *Robert A. Miller*  
*Oscar L. Spencer.*

ATTORNEY

2,750,332

**METHOD AND APPARATUS FOR ELECTRO-DEPOSITION OF A LAYER OF UNIFORM THICKNESS ON A CONDUCTIVE SURFACE**

Robert A. Miller, Tarentum, Pa., assignor to Pittsburgh Plate Glass Company, Allegheny County, Pa., a corporation of Pennsylvania

Application June 4, 1952, Serial No. 291,609

6 Claims. (Cl. 204—15)

This invention relates to a method and apparatus for the electro-deposition of a metallic layer of constant thickness upon an electrically conductive surface and more particularly for the electro-deposition of a thin copper plating or film upon a silver film which has been deposited on glass to form a mirror, the copper film acting as a protective coating on the silver film.

It has been difficult if not impossible to cover a thin primary film or sheet of the thickness of a silver film used for mirrors, with a uniform outer film of copper or other suitable metal by existing electrolytic processes. Non-uniformity in the thickness of the deposited outer film results from the relatively high electrical resistance of the thin primary film.

For example, one prior method of applying the outer copper film has been to hold the mirrored glass plate stationary in a bath of copper sulphate with copper anode bars suspended in the solution approximately 4 inches from the silvered surface. The silver film was connected to the opposite pole of the system by means of suitable electrical contacts to constitute the cathode. The bath was usually a highly acid saturated solution of copper sulphate; the current density approximately 3 amperes per square foot at 1.5 volts, and the plating time was approximately 3 minutes. The copper coating varied from a heavy layer at the edges of the mirror where the clamps were attached, about the periphery, to essentially no sensible thickness at the center, remote from the contacts, on a reasonably large mirror. At the edges of the plate, the weight of copper might run as high as 0.50 gram per square foot or a thickness of 0.000024 inch, whereas, at the center the weight of copper may approach 0.08 gram per square foot, or a thickness of 0.000004 inch, or less.

A principal object of this invention, therefore, is to provide a method and apparatus by which an outer or protective metal film of uniform thickness may be applied to a thin primary film on a large surface such as the silver film on a mirror.

A certain degree of uniformity of rate of deposition of the secondary film may be achieved by providing a plating bath vessel of conical or pyramidal shape in which the anode is positioned at the apex of the cone or pyramid with the primary film as the cathode at the base of such cone or pyramid. The shape of the plating bath would have to be carefully calculated and might have to be re-proportioned for primary films of different sizes and shapes.

Another method of obtaining uniform deposition is to dispose electrical contacts at a plurality of points on the primary film but such a method would not be desirable for use in the case of mirror films for the contacts would damage the primary silver film and defeat the purpose of applying a protective coating to the primary film.

The method and apparatus of this invention eliminates the immersion of the glass and primary film. Instead, the glass with the electrically conductive silver

film is supported and conveyed past an electro-deposition station. The electrolyte solution is contained in a supply tank at the station. A positive electrode is disposed in the tank and immersed in the solution. A nozzle outlet or applying means is connected to the tank and is arranged to feed a stream of electrolyte onto the primary film across the width of the film. The negative electrical contacts are made along the edge of the primary film which is to pass through the deposition station first.

10 In operation, with the positive and negative electrodes suitably connected to a source of power, the stream of electrolyte is fed first onto the primary film at the edge where the cathode contacts are placed. The electric current between the anode metal in the electrolyte tank and the cathode contacts on the primary film is maintained by the continuous flow of the electrolyte onto the primary film. As a result, the anode metal is deposited on the primary film along the edge near the contacts on the primary film. The movement of the glass and the primary film is such that the desired thickness is applied first along that edge, and then as the glass and the primary film is moved at a uniform speed the edge of the primary film along which the cathode contacts are made moves away from the electrolyte feeding means in the deposition station. As the glass and primary film move through the station, successive areas of the primary film will thus be covered with electrolyte and the outer metal will be deposited in such areas. A receiving tank below the deposition station serves to collect the spent solution.

For a more complete description of the invention, reference is made to the drawings, wherein:

Fig. 1 is a schematic side view of one form of apparatus embodying the invention;

Fig. 2 is a view partly in section, taken along the line 2—2 in Fig. 1;

Fig. 3 is a perspective view of a glass plate showing the relationship of the primary and the outer films.

Fig. 4 is a longitudinal cross sectional view of an alternate form of electrolyte feeding nozzle;

Fig. 5 is a bottom plan view of the alternate form of nozzle shown in Fig. 4.

The apparatus illustrated in the drawings includes a conveyor such as a roller conveyor 10, illustrated schematically in Fig. 1, having rollers 11 for supporting a glass plate 12. The plate 12 has a primary film 13 upon one face. The glass is oriented with the silver film uppermost.

50 A supply tank or container 15 suitable for receiving an electrolytic solution 16 may be positioned, above the glass, in any suitable manner. A nozzle 17 is provided which is connected to the tank 15 by suitable means such as connecting hose 18.

The nozzle 17 may be of a size to extend across the width of the glass mirror being treated. The lower side of the nozzle may be formed to define a plurality of small diameter apertures 20 through which electrolyte may be fed onto the primary film 13.

60 At least one anode or positive electrode 21 of the metal to be plated may be immersed in the supply tank 15.

A primary film 13 forms the cathode or negative electrode, electrical contact to the film being made by suitable means such as one or more alligator clips 22 along one 65 end of the glass.

In operation, initially, a stream of electrolyte is fed from the solution supply tank 15 onto the primary film adjacent the alligator clips 22 until the desired thickness of the outer film metal has been deposited on the primary film in the area around the clips. Thereafter, the glass 12 is moved, as indicated by the arrow in Fig. 1, from right to left, so that there is a uniform deposition

of the outer film at progressively remote areas from the cathode contacts at the end of the primary film. A receiving tank 23 may be provided below the glass plate 12 in the general area of the nozzle 17 to recover the used electrolyte solution. A suitable drain 25 may be provided for drawing the solution from the receiving tank.

Electric current flows through the apparatus only when the stream of electrolyte is flowing upon the primary film. The thickness of the secondary film will depend upon the current density at the electrolyte nozzle 17, upon the rate at which the primary film is moved past the nozzle, also upon the concentration of cations in the electrolyte and upon the temperature.

As a guide to the variables effecting the thickness of the deposition of the outer film, it has been found that various copper sulphate solutions may be used ranging from one of high acidity such as pH 1.5, to one of high alkalinity such as pH 8 or 9. More rapid deposition is obtainable from reasonably high acidity than from either neutral or alkaline solutions, whereas a brighter looking copper film is obtained from a neutral or slightly alkaline solution. The copper sulphate bath should be a nearly saturated solution. The pH value in the solution can be controlled by the addition of  $H_2SO_4$  to lower the pH or the addition of a suitable buffer solution to raise the pH.

The current density may vary from approximately 1.5 amperes to 5 or 6 amperes per square foot at a voltage of from 1.5 to 5, the area to be considered being that of the solution-dispensing nozzle, carrying the current and the copper solution to the primary film. The desired current density and voltage may be readily determined.

As an example, at a current density of 3 amperes over a nozzle area of 12 square inches, with a voltage of 1.5, and a forward motion of the plate at a rate of 12 inches per minute, the copper film thickness resulting is approximately 0.000008, or a weight of .178 gram of copper per square foot. The amount of copper deposited will vary directly with the amperage and voltage and inversely with the speed of forward movement of the plate being coated.

The temperature of the solution should normally be maintained at about 70° to 75° F. If the solution is colder, the amount of copper deposited will be less, although it will be more firmly bonded and brighter. If the solution is warmer, the amount of copper deposited will be greater, however, it will be less firmly bonded and more porous.

In the apparatus illustrated, the nozzle 17 shown in Fig. 2 is arranged to extend across the entire width of the mirror and the outlet means may be 72" in length to span the entire width of a large mirror. It will be appreciated that conventional overhead supports (not shown) along the length of the nozzle may be provided to support it. The nozzle is spaced very close to the surface of the primary film but the supports for the nozzle and the glass should be such that the nozzle does not come in contact with the primary film at any time.

Figs. 4 and 5 illustrate an alternate form of nozzle 35 having a single slit aperture 36 and having felt members 37 on both sides of the aperture 36 to confine the electrolyte solution 38 being fed from the nozzle 35 onto the primary film 40 on the glass 41. It will be noted from Fig. 4 that the lower faces of the felt members 37 are maintained out of contact with the primary film to prevent injury to such film but effectively confine the electrolyte to the plating area.

Although for simplicity of showing the cathode or negative contacts are illustrated as clips 22 in contact with the upper surface of the primary film 13 and also in contact with the deposited outer film 14, in practice, it may be preferred to contact the silver coating which extends over the leading edge of the glass, as shown in Fig. 3 so that no portion of the mirror surface of the primary film is damaged. The cathode connection may

5 be a line contact 24 in electrical engagement with the most uniform and economical plating with the highest deposition of copper, the line contact should remain in fixed position on the edge of the mirror and move forward with it.

It will be appreciated from the foregoing that the method and apparatus of this invention fulfills the objects of applying a thin outer film of uniform thickness to a thin primary film.

10 In accordance with the provisions of the patent statutes, I have herein described the principle of operation of the invention, together with the elements which I now consider the best embodiments thereof, but I desire to have it understood that the structure disclosed is only illustrative and the invention can be carried out by other means. For example, whereas, in the illustrated embodiment of the invention the glass containing the mirror to be coated is moved while the nozzle means for feeding the electrolyte is stationary, it will be appreciated that a moving nozzle with respect to a stationary mirror is also contemplated within the scope of the invention. Also, while it is designed to use the various features and elements in the combinations and relations described, some of these may be altered and modified without interfering with the more general results outlined.

15 Having thus described my invention, I claim:

1. In apparatus for the electro-deposition of a metallic layer of constant thickness upon an electrically conductive surface having a conveyor adapted for supporting and conveying the said surface along a predetermined path and past an electro-depositing station for presenting successive areas of the conductive surface at said station, a supply tank containing an electrolytic bath, a positive electrode disposed in the supply tank and immersed in the bath, an applicator connected to said supply tank, a negative electrode connected to the electrically conductive surface and with the electrolyte on said surface, and means to connect a source of electricity to the positive and negative electrodes, said applicator comprising a nozzle for projecting said electrolyte onto the conductive surface at said station, and including depending means attached to the edges of said nozzle, said applicator being mounted at said station and relative to said conveyor so that said depending means substantially confines the electrolyte to said station without contacting said conductive surface.

2. In apparatus for the electro-deposition of a metallic layer of constant thickness upon an electrically conductive surface having a conveyor adapted for supporting and conveying the said surface along a predetermined path and past an electro-depositing station for presenting successive areas of the conductive surface at said station, a supply tank containing an electrolytic bath, a positive electrode disposed in the supply tank and immersed in the bath, an applicator connected to said supply tank, a negative electrode connected to the electrically conductive surface and with the electrolyte on said surface, and means to connect a source of electricity to the positive and negative electrodes, said applicator comprising an elongated nozzle extending over the full width of said station transversely to said predetermined path and having a slit centrally located therein for projecting said electrolyte onto the conductive surface at said station, said nozzle also including depending absorbent material means attached to and extending continuously around the edges of said nozzle, said applicator being mounted at said station and relative to said conveyor so that said depending means substantially confines the electrolyte to said station without contacting said conductive surface.

3. In apparatus for the electro-deposition of a metallic layer of constant thickness upon an electrically conductive surface having a conveyor adapted for supporting and conveying the said surface along a predetermined

primary film across the entire width of the mirror. For path and past an electro-depositing station for presenting successive areas of the conductive surface at said station, a supply tank containing an electrolytic bath, a positive electrode disposed in the supply tank and immersed in the bath, an applicator connected to said supply tank, a negative electrode connected to the electrically conductive surface and with the electrolyte on said surface, and means to connect a source of electricity to the positive and negative electrodes, said applicator comprising an elongated nozzle extending over the full width of said station transversely to said predetermined path and having a slit centrally located therein for projecting said electrolyte onto the conductive surface at said station, said nozzle also including depending absorbent material means attached to and extending continuously around the edges of said nozzle for substantially confining the electrolyte to said station, said applicator being mounted at said station and relative to said conveyor so that said depending means substantially confines the electrolyte to said station without contacting said conductive surface.

4. In apparatus for the electro-deposition of a metallic layer of constant thickness upon an electrically conductive surface having a conveyor adapted for supporting and conveying the said surface along a predetermined path and past an electro-depositing station for presenting successive areas of the conductive surface at said station, a supply tank containing an electrolytic bath, a positive electrode disposed in the supply tank and immersed in the bath, an applicator connected to said supply tank, a negative electrode connected to the electrically conductive surface and with the electrolyte on said surface,

and means to connect a source of electricity to the positive and negative electrodes, said applicator being mounted at said station and comprising an elongated nozzle extending over the full width of said station transversely to said predetermined path and having a slit centrally located therein for projecting said electrolyte onto the conductive surface at said station, an absorbent material edge depending from the nozzle and surrounding said slit, said edge extending close to the conductive surface for confining said electrolyte to said station but maintaining a clearance to avoid contact with said conductive surface.

5. The invention according to claim 4 wherein said absorbent material edge is relatively thick to provide good absorbing capacity.

6. The invention according to claim 5 wherein said absorbent material edge is constructed of felt.

References Cited in the file of this patent

UNITED STATES PATENTS

|           |               |       |               |
|-----------|---------------|-------|---------------|
| 883,756   | Steiner       | ----- | Apr. 7, 1908  |
| 1,416,929 | Bailey        | ----- | May 23, 1922  |
| 1,582,407 | King          | ----- | Apr. 27, 1926 |
| 1,603,951 | Hitchcock     | ----- | Oct. 19, 1926 |
| 1,771,680 | Ishisaka      | ----- | July 29, 1930 |
| 1,809,826 | Bohlman       | ----- | June 16, 1931 |
| 2,540,602 | Thomas et al. | ----- | Feb. 6, 1951  |

FOREIGN PATENTS

|               |       |               |
|---------------|-------|---------------|
| Great Britain | ----- | of 1896       |
| Great Britain | ----- | Mar. 22, 1928 |
| Sweden        | ----- | Dec. 15, 1915 |